

June 17, 1952

W. D. BALDSIEFEN

2,600,831

LIGHT-SENSITIVE SILVER HALIDE PHOTOGRAPHIC ELEMENTS

Filed July 26, 1949



FIG. 1.



FIG. 2.



FIG. 3.



FIG. 4.



FIG. 5.

INVENTOR.  
WALTER DEWEY BALDSIEFEN  
BY

*Lynn Barrett Morris*

ATTORNEY

UNITED STATES PATENT OFFICE

2,600,831

## **LIGHT-SENSITIVE SILVER HALIDE PHOTOGRAPHIC ELEMENTS**

Walter Dewey Baldsiefen, Metuchen, N. J., assignor to E. I. du Pont de Nemours and Company, Wilmington, Del., a corporation of Delaware

Application July 26, 1949, Serial No. 106,962

6 Claims. (Cl. 95—8)

1

The invention relates to photographic elements, an outer water-permeable layer or stratum of which has improved surface characteristics. More particularly, it relates to photographic films and papers which have an outer light-sensitive, anti-abrasion and/or non-halation layer which has improved surface characteristics and other useful properties. It also relates to a process of coating photographic films and papers.

Photographic films and papers are generally manufactured in the form of continuous sheets or webs which are provided with various coatings from predominantly aqueous solutions. The coatings are dried by passing the coated web through a chamber maintained at an elevated temperature. This is generally accomplished by festooning so that the length of the chamber can be kept within reasonable limits. The coatings which generally consist of a water-permeable colloid which serves as a binding agent for the silver halides, anti-halation dyes or pigments, etc., are quite smooth and when the film or paper is again passed through the drying chamber with the coated surface in contact with the festooning supports, tend to slip with damage to the coated sheet or web. Saponin is generally used in the coating solutions in order to facilitate the spreading of the coatings, but it is not always uniform in properties and what is more serious washes out during photographic processing operations which causes "water-spots" which are caused by non-wetting by subsequent processing baths. These water spots which are present in negative films, etc., seriously affect the quality of the resulting positive prints. Various surface active wetting agents have been proposed to facilitate spreading of gelatin silver halide layers, antihalation layers and the like but they render the surfaces smooth so that slipping on the festooning supports becomes a real problem.

An object of this invention is to improve the art of coating continuous lengths of photographic films and papers. A further object is to provide coatings for photographic elements which have improved non-slipping surface characteristics. A still further object is to provide photographic elements with water-permeable coatings which have good uniform rewetting characteristics. Still other objects will be apparent from the following detailed description of the invention.

It has been found that improved photographic films and papers can be made by incorporating

2

in an outer water-permeable colloid light-sensitive silver halide layer, a water-permeable colloid anti-abrasion layer on a water-permeable backing or anti-halation layer or in a plurality of 5 such layers a salt of an alkyl-substituted aryloxy alkylene ether sulfonate of the general formula:



10 where R is an alkyl radical of 4 to 12 carbon atoms, n is a cardinal number from 1 to 2 and M is an alkali metal or ammonium. R may be straight chain or branched chain butyl, amyl, hexyl, heptyl, octyl, nonyl or decyl. The radical n is preferably 1 and R p-tertiary octyl.

The compounds of the above formula are preferably added to the aqueous coating solution in an amount of about 0.1 to 5.0% based on the colloid in the solution prior to coating of the layer in question. The coatings may then be applied in any of the conventional manners.

The invention will be further illustrated but is not intended to be limited by the following examples.

*Example 1*

A coating solution for a non-halation backing layer was prepared by dissolving 400 grams of gelatin and 15 grams of nigrosine (Colour Index 30 No. 865) in sufficient water to make 10 liters. To this solution there was added 5 grams of sodium p-tertiary-octyl phenoxy ethoxy ethyl sulfonate of the formula:



This material was then coated onto a cellulose acetate film base 1 as shown in Fig. 1 of the drawing to form non-halation layer 2 which was dried in the manner known to the art. A gelatin-silver halide emulsion layer 3 was then coated from an aqueous dispersion on the opposite surface of the support. During this latter operation no difficulty was encountered with the film slipping from the festooning supports, due to slipperiness of the non-halation layer.

*Example 11*

50 A gelatino-silver halide emulsion layer 5 was  
coated onto a cellulose acetate film base 4 as  
shown in Fig. 2 of the drawing and dried. To  
10,000 grams of an anti-abrasion overcoating  
55 solution containing 200 grams of hard gelatin  
dissolved in 9,800 grams of water, there was added

2 grams of sodium p-tertiary octylphenoxy ethoxy ethyl sulfonate having the formula given in Example I and the resulting solution was coated onto the silver halide emulsion layer to form anti-abrasion layer 6 and dried. A sample of this material was then exposed and processed in a developing bath containing 2 grams of metol, 5 grams of hydroquinone, 100 grams of sodium sulfite and 6 grams of borax dissolved in sufficient water to make a total volume of the solution 1 liter. It was observed that the material could be rapidly plunged into the solution without the formation of air bubbles on the emulsion surface, and that the solution wet said surface completely, thus obviating the formation of water-spots in the processed material.

*Example III*

A continuous length of photographic film prepared as in Example II was coated on the back side with another gelatino-silver halide emulsion layer, and passed through a drying chamber. This film is shown in Fig. 3 of the drawing and consists of cellulose acetate film base 4 which has superimposed on one surface gelatin silver halide emulsion layer 5 on which is superimposed gelatin layer 6 containing sodium p-tertiary, octyl phenoxy ethoxy ethyl sulfonate and on the reverse side of the film base is gelatin silver halide layer 7. During this latter coating operation no difficulty was encountered because of slippage of the material during its travel in festoons through the drying.

*Example IV*

To 10,000 grams of a gelatino-silver halide emulsion containing approximately 1600 grams of solids there was added 8 grams of sodium p-tertiary octylphenoxyethoxyethyl sulfonate having the formula set forth in Example I; the emulsion was then coated on a cellulose film base 8 as shown in Fig. 4 of the drawing in the manner known in the art to form layer 9. It was observed that the emulsion coated smoothly and with uniform adherence to the base. It was found that the emulsion surface was wetted instantly during the processing operations, and that no spots were visible when the processed film was finally dried.

*Example V*

A continuous length of cellulose acetate film base 2 as shown in Fig. 5 of the drawing was coated on its back surface with an aqueous solution made by dissolving 400 grams of gelatin, 15 grams of nigrosin in sufficient water to make 10 liters of solution. To this solution there was added 1.2 grams of glycoxal and 5 grams of sodium p-tertiary-octyl-phenoxy ethoxy ethyl sulfonate having the formula set forth in Example I and resulting layer 1' was dried in a tunnel provided with festooning supports. The front surface of the film base was then coated with a silver iodobromide emulsion layer 3 from a solution of the type described in Example II and dried in like manner. The film had the advantage that the surfaces did not slip on the festooning supports. In addition, the sodium p-tertiary octylphenoxy ethoxy ethyl sulfonate did not wash out during processing and resulted in negative pictures which were free from "water spots." The glycoxal, moreover, prevented reticulation of layer 1' during processing.

The above coatings were made under conditions that no actinic light exposed the light-sensitive silver halide coatings.

In place of the specific anti-halation dye of the foregoing examples there may be substituted one or more other dyes or pigments or colloidal silver. The particular dye or dyes, etc., used depends on the characteristics of the emulsion. The anti-halation material should be absorptive of light of wavelengths to which the emulsion is sensitive. Suitable additional dyes include:

- 10 Auramine (C. I. 655)
- 10 Helianthin (C. I. 142, 146)
- 10 Brilliant yellow S (C. I. 144)
- 10 Chrysoin (C. I. 148)
- 10 Acid blue black (C. I. 246)
- 15 Rhodamine (C. I. 749, 750, 751, 746, 753, 761, 763)
- 15 Fuchsin (C. I. 677)
- 15 Safranine G (C. I. 841)
- 15 Ponceau 6R (186)
- 15 Crocein scarlet (C. I. 277, 251, 286, 252, 291, 183)
- 20 Azorubin (C. I. 179)
- 20 Safranine O (C. I. 841)
- 20 Ponceau 2R (C. I. 79)
- 20 Spirit soluble nigrosine (C. I. 864)
- 20 Metanil yellow (C. I. 138)
- 25 Acid magenta O (C. I. 692)

The C. I. numbers in the foregoing table refer to Colour Index numbers, the Colour Index being the Society of Dyers and Colourists Colour Index, edited by F. M. Rowe, published by the society, 30 Bradford, Yorkshire, England.

Similarly in place of gelatin as the water-permeable colloid other such materials may be used. Among such materials are albumin, casein, agar agar, polyvinyl alcohol, hydrolyzed ethylene/vinyl acetate copolymers, polydioxolanes, etc.

The invention is not limited to the use of cellulose acetate film base as stated above, but can be used with practically any type of transparent film or paper e. g., baryta or resin coated paper; or film composed of polyamides, cellulose nitrate, polyvinyl acetals, cellulose propionate, cellulose mixed esters, cellulose ethers, vinyl chloride and copolymers, styrene, acrylonitrile and copolymers, polyesters, vinyl acetate and copolymers, vinyl fluoride and copolymers, polyvinyl alcohol; transparentized paper, etc.

Sensitizing dyes and other emulsion adjuvants may be added to the above emulsion layers without their function being affected by the alkyl substituted aryloxy alkylene ether sulfonates. This is particularly advantageous in the case of the so-called dupli coated photographic elements, where an emulsion layer may be sensitized to one portion of the spectrum, while the emulsion layer 55 on the opposite side of a film base may be sensitized to another portion of the spectrum, or may not be especially sensitized at all. The agents of Formula I are included in at least one, and preferably both of the emulsion layers, to facilitate coating and subsequent processing. The principal advantage of the invention, however, is that it allows the manufacture of such a double coated element, without the danger of waste caused by the element slipping off from the festooning supports on to the floor of the drying tunnels.

A further advantage over saponin is that uniform results can be obtained. The former being a naturally occurring material often varies in properties.

As many widely different embodiments of this invention can be made without departing from the spirit and scope thereof, it is to be understood that the invention is not to be limited except 75 as defined by the claims.

What is claimed is:

1. A photographic element comprising a support and a light-sensitive silver halide emulsion layer said element having at least one water-permeable outer layer which contains a small amount of a compound of the formula:



wherein R is an alkyl radical of 4 to 12 carbon atoms, n is a cardinal number from 1 to 2 and M is a member taken from the group consisting of alkali metals and ammonium.

2. A photographic element comprising a support and a light-sensitive silver halide emulsion layer said element having at least one water-permeable outer layer which contains a small amount of a compound of the formula:



3. A photographic element comprising a transparent flexible film base bearing a light-sensitive colloid silver halide emulsion layer, a water-permeable colloid anti-abrasion layer on said emulsion layer and a layer of a water-permeable colloid containing an anti-halation material on the reverse surface of the base at least one of the latter two layers containing a small amount of a compound of the formula:



wherein R is an alkyl radical of 4 to 12 carbon atoms, n is a cardinal number from 1 to 2 and M is a member taken from the group consisting of alkali metals and ammonium.

4. A photographic element comprising a transparent flexible film base bearing a light-sensitive

colloid silver halide emulsion layer, a water-permeable colloid anti-abrasion layer on said emulsion layer and a layer of a water-permeable colloid containing an anti-halation material on the reverse surface of the base at least one of the latter two layers containing a small amount of a compound of the formula:



5. A photographic element comprising a transparent flexible film base bearing a gelatino silver iodobromide emulsion layer on one surface, a gelatin anti-abrasion layer on said emulsion layer and a layer of gelatin containing an anti-halation material on the reverse surface of the base each of the two latter layers containing a small amount of a compound of the formula:



and a small amount of glyoxal.

6. An element as set forth in claim 5 wherein the anti-halation material is acid Magenta O.

WALTER DEWEY BALDSIEFEN.

#### REFERENCES CITED

The following references are of record in the file of this patent:

#### UNITED STATES PATENTS

| 35 | Number    | Name          | Date          |
|----|-----------|---------------|---------------|
|    | 1,946,635 | Murray et al. | Feb. 13, 1934 |
|    | 2,115,192 | Bruson        | Apr. 26, 1938 |
|    | 2,118,059 | Slack et al.  | May 24, 1938  |
|    | 2,143,759 | Bruson        | Jan. 10, 1939 |
| 40 | 2,287,807 | Kendall       | June 30, 1942 |
|    | 2,400,532 | Blake         | May 21, 1946  |